

Jan. 9, 1951

R. D. OPPENHEIM

2,537,785

METHOD OF PROTECTING SHOES DURING MANUFACTURE

Filed Jan. 6, 1949

2 Sheets-Sheet 1



INVENTOR.  
RICHARD D. OPPENHEIM  
BY  
*Moche Blum*  
ATTORNEYS.

Jan. 9, 1951

R. D. OPPENHEIM

2,537,785

METHOD OF PROTECTING SHOES DURING MANUFACTURE

Filed Jan. 6, 1949

2 Sheets-Sheet 2

*Fig. 3*



*Fig. 4*



INVENTOR.

RICHARD D. OPPENHEIM

BY

*Mock & Blum*

ATTORNEYS.

## UNITED STATES PATENT OFFICE

2,537,785

METHOD OF PROTECTING SHOES DURING  
MANUFACTURERichard D. Oppenheim, Woodside, N. Y., assignor  
to Spraylat Corporation, New York, N. Y., a  
corporation of New York

Application January 6, 1949, Serial No. 69,511

5 Claims. (Cl. 12—142)

1

My invention relates to the manufacture of shoes, and has particular reference to a method of removing temporary protective coatings from a portion of the upper.

In the manufacture of shoes, it has been found desirable to provide a film of latex or a latex composition on the outer surface of the shoe upper. This application is beneficial to the appearance and quality of the finished shoe in that it is applied before lasting and protects the upper from soilage due to sole cement, dyes, and other ingredients used in shoe manufacture. The composition of such latex protective materials, as well as the method for applying the same to a shoe, are both well-known and are adequately described in such patents as Patent No. 1,924,214 issued to Edwin B. Newton, and Patent No. 2,049,554 issued to Walter H. Wedger.

The manufacture of shoes according to the aforementioned methods, is, however, subject to several disadvantages. Before the outsole of the shoe may be cemented to the insole, the marginal edge portion of the upper overlying the insole must be roughened or abraded, and therefore must be first cleared of any protective film. It is extremely important, however, to protect the exposed outer edge of the upper against soilage due to the sole cement as well as the dyes used on the outsole. The lower edge of the upper, adjacent the lasting portion must particularly be protected against soilage. It is important, therefore, to remove the film from the marginal area, while retaining it upon the rest of the upper. In order to cleanly strip the film from the finished shoe, no portion of the film should remain between the outsole and the upper.

Due to the elastic nature of the rubber film, it is impossible to remove by roughing the unwanted section of film on the marginal edge portion of the upper overlying the insole without tearing or otherwise damaging the latex coating on the adjacent portions of the upper.

There have been various methods proposed for removing unwanted portions of the latex protective covering while retaining the desired protective coating intact and undamaged. The most satisfactorily-proven method up to the present has been the use of a dull, hot knife with which the undesired latex portions are scored off. The marginal area of film may then be stripped off, permitting the shoe to be roughened on this area. This process of scoring with a cautery knife is, however, time-consuming and introduces a new operation in the shoe manufacturing process. Another method of meeting this problem is sug-

2

gested in the aforementioned Patent No. 2,049,554 and comprises applying the latex composition to the outsole by means of a brush after the outsole has been attached to the last. This method has been found undesirable since it is more expedient to apply the latex coating to the outsole before the lasting step is reached.

It is the principal object of my invention, therefore, to provide a novel method for removing any desired portion of a temporary protective latex film without interfering with the normal shoe manufacturing process.

Another object of my invention is the provision of a novel method of roughening the marginal lasting portion of the shoe upper without tearing or otherwise damaging the adjacent protective coating.

Still another object of my invention is the provision of a protective coating for shoes which will not readily rupture upon contact with shoe-machine parts.

These and other objects of my invention will be readily apparent in the course of the following specification when taken in connection with the accompanying drawings, in which:

Fig. 1 is a bottom perspective view of a shoe attached to the last, and treated with a lacquer coating according to my new method;

Fig. 2 is a fragmentary section thereof, taken along line 2—2 of Fig. 1;

Fig. 3 is a bottom perspective view similar to Fig. 1 but showing the lacquer-treated latex coating removed from the marginal lasting portion of the upper; and

Fig. 4 is a fragmentary section taken along line 4—4 of Fig. 3.

The drawings illustrate a cement shoe, by which is meant a shoe to which the outsole is to be cemented. The shoe comprises an upper 11 which has been covered by an outer film of protective latex or latex composition 12, as previously described. The entire upper 11 may be covered with the latex film 12 before lasting. The upper 11 is then attached to a conventional last 10 in the usual manner.

To the latex film 12 which covers the marginal overlapping lasting portion M of the upper, an outer coating of film-forming lacquer 13 is applied. The said lacquer 13 may be applied with a brush or in any other suitable manner. The marginal overlapping lasting portion M of the upper to which the lacquer is applied, is that portion of the upper 11 which overlies the top surface of the last 10, and which must be roughened before the sole is cemented thereto. The

lacquer is also applied to the adjacent areas of the upper, for reasons which will be presently set forth.

The lacquer which has low elongation, high tensile strength, and good adhesion, bonds to the latex film and forms with said latex film a single bonded, tough film which is rigid enough to be severed and removed by means of a rotating roughing wheel. Figs. 1 and 2 show the lacquer film 13 applied to the latex coating 12 on the marginal lasting portion of the upper 11 and also on the adjacent areas on the sides of said upper 11.

After the lacquer has dried sufficiently to form a tough and rigid bonded film 13 on the latex coating 12, lacquer film 13 and its bonded latex film 12 are abraded from the marginal overlapping lasting portion M of the upper 11. The abrading may be done by means of a conventional rotating roughing wheel, and thus the unwanted area of latex film may be removed and the marginal lasting portion M of the upper roughened in the same operation.

Figs. 3 and 4 show the lasted upper 11 after the bonded film of latex 12 and lacquer 13 on the marginal lasting portion has been removed by the roughing wheel, leaving the upper 11 exposed. Since the adjacent areas are also covered with the lacquer, the marginal portion of latex and lacquer may be cleanly severed without tearing or rupturing the adjacent areas of latex.

The lacquer film 13 has no permanent deleterious effect upon the rubber latex film 12, and does not in any way interfere with its removal after the shoe is finished.

After the marginal portion has been roughened, the adjacent areas remain covered with lacquer, which forms a hard, smooth, tough outer coating on the latex film, preventing it from rupturing from friction of machine parts. Because of this tough outer coating, a machine part, such as an edge trimmer shield may be slid along the lower portion of the upper or otherwise brought into contact therewith, without damaging the coating or impairing its protective function.

In the drawings, the lacquer-covered latex is shown abraded and removed from the entire area of the upper overlapping the top of the last. If desired, however, the latex on the heel portion of this area may be left on the upper, since the heel is not cemented to the shoe. Instead of abrading the latex off the upper in this area, it is merely necessary to abrade a narrow line between the marginal portion and the adjacent area. This may be done by the use of a small emery wheel, or in any other desired manner. The heel may thus be attached directly over the latex and lacquer film in the respective marginal portion, and when the shoe is finished, the protective latex may be cleanly stripped from the remainder of the upper, because of the abraded line.

The method described in the next preceding paragraph is particularly useful in the manufacture of welt shoes and the combination welt and cement shoes, in which it is only necessary to remove the protective film from a small area between the upper and outsole which is to be cemented. Thus the latex covering on the welt portion of the overlapping upper may be severed or cut from the remaining portion of the latex covering, by making a narrow line between the two portions with an emery wheel. The sole

may be attached over the separated portion of latex on the overlapping upper and the remaining portion of latex covering on the upper cleanly stripped off, after the shoe is finished.

The aforementioned lacquer which is applied to the protective latex portion may be formulated from any of the film-forming resins such as ethyl cellulose, cellulose acetate, cellulose nitrate, or polyvinyl resins. Such resins may be used alone, or may be combined with plasticizers and natural or synthetic resins.

I have found that the best results for efficient shoe manufacturing may be obtained by the use of a lacquer which is easy to apply and fast-drying, and which has good film strength as well as good adhesion. By adding rapid-drying solvents to the lacquer, the lacquer can be applied to the upper at any time after the lasting operation without interfering with the normal plant operation by requiring operations to be suspended while the lacquer is drying. I have found that best results may be obtained by using the compound made according to the following formula:

|    | Parts by weight                                    |    |
|----|----------------------------------------------------|----|
| 25 | Ethyl cellulose (Dow Chemical Standard<br>100 cp.) | 10 |
|    | Toluol                                             | 80 |
|    | Ethyl alcohol                                      | 20 |

30 Toluol or other similar rubber solvent is used in the lacquer primarily as a solvent for the ethyl cellulose, but also for its effect upon the latex coating. The toluol combines with the latex film which is covered by the lacquer, reducing the elastic qualities of the latex. The latex coating in the presence of toluol, swells and becomes weakened, having a low elongation. Thus the weakened layer of latex and its bonded layer of lacquer offer a surface which may be easily abraded. After a relatively short period, the toluol will evaporate leaving the protective latex coating with its elasticity unaffected. The latex coating may then be conveniently peeled from the upper.

35 40 45 50 55 The use of fast-drying solvents such as ethyl alcohol and toluol provide reagents of such rapid-drying properties, that within fifteen minutes after application, the lacquer and its bonded latex may be removed from the marginal area of the upper by roughing. Thus the compound may be applied immediately after the bottom ironing of the marginal area without loss of appreciable time of manufacture.

55 60 65 70 Should the manufacturing process be such that drying time is not a critical factor, it is possible to use a water solution or a water dispersion of film-forming materials, such as polyvinyl alcohol, polyvinyl butyral, methyl cellulose, and casein. These materials possess all of the aforementioned desired qualities, except that they are relatively slow-drying.

75 It is obvious that numerous alterations, additions and omissions may be made in my invention without departing from the spirit and scope thereof. For example, the lacquer may be applied to any desired portion of the latex covering on the upper, instead of the marginal lasting portion.

I claim:

70 75 1. A method of protecting shoes during manufacture which comprises applying a latex coating to a shoe upper, assembling said shoe upon a last, applying to portions of said latex covering a film-forming lacquer which will bond to said latex coating to form a rigid covering on

the shoe upper, then abrading selected portions of said rigid covering from the shoe upper while leaving the remainder of the latex coating unaffected, proceeding with the lasting operation, and subsequently stripping the remainder of the latex coating from the upper.

2. A method of protecting shoes during manufacture which comprises applying a latex coating to a shoe upper, assembling said shoe upper on a last, applying to the marginal edge portion of the upper a film-forming lacquer which will bond to said latex coating to form a rigid covering on said marginal edge portion, then abrading the rigid covering from said marginal edge portion while leaving the coating on the remainder of the upper unaffected, attaching the outsole of the shoe over the marginal edge portion of the upper, and subsequently stripping the remaining latex covering from the shoe upper.

3. A method of protecting shoes during manufacture which comprises applying a latex coating to a shoe upper, assembling said shoe upper on a last, applying to the marginal edge portion of the lasted upper a film-forming lacquer which is made of a resin and a rubber solvent and which will combine with the latex coating to form a rigid, non-elastic outer coating on said marginal edge portion, then abrading the rigid outer coating from said marginal edge portion while leaving the coating on the remainder of the upper unaffected, and simultaneously roughening the marginal edge portion of the shoe upper, attaching the outsole of the shoe over the roughened portion of the upper, and subsequently stripping the remaining latex covering from the shoe upper.

4. A method of protecting shoes during manufacture which comprises applying a latex coating over the entire surface of a shoe upper, assembling said shoe upper on a last, applying to the marginal edge portion of the lasted upper a film-forming lacquer composed of a film-forming resin, a rubber solvent, and a rapid drying agent, allowing said lacquer to dry sufficiently to combine with said latex coating and to form a non-elastic rigid film therewith, abrading said rigid film from the marginal edge portion of the shoe upper with a roughening wheel and simultaneously roughening the marginal edge portion of the shoe upper while leaving the coating on the remainder of the shoe upper unaffected, attaching the outsole of the shoe over the roughened portion of the upper, and subsequently stripping the remaining latex covering from the shoe upper.

5. A method according to claim 4 in which the areas of the shoe upper adjacent the marginal edge portion are also coated with the film-forming lacquer, and in which said lacquer is left upon the latex covering until the latex covering is stripped from the upper.

RICHARD D. OPPENHEIM.

#### REFERENCES CITED

The following references are of record in the file of this patent:

#### UNITED STATES PATENTS

| Number    | Name             | Date          |
|-----------|------------------|---------------|
| 1,339,462 | Lionne           | May 11, 1920  |
| 2,031,674 | Schneider et al. | Feb. 25, 1936 |